# EUROPEAN PATENT SPECIFICATION

(11) **EP 2 655 731 B1**
(45) Date of publication and mention of the grant of the patent: **08.05.2019**
(21) Application number: 11851854.7
(22) Date of filing: 16.12.2011
(51) Int. Cl.: D21C 3/22, D21C 7/12

(54) **A METHOD OF CONTROLLING A PULPING PROCESS IN A FEED-FORWARD MANNER**
VERFAHREN ZUR STEUERUNG EINES AUFSCHLUSSVERFAHRENS IN EINEM VORWÄRTSKOPPLUNGSVERFAHREN
PROCÉDÉ DE COMMANDE D'UN PROCESSUS DE FABRICATION DE PÂTE À PAPIER DE MANIÈRE PRÉDICTIVE

(30) Priority: 22.12.2010 SE 1051361
(43) Date of publication of application: 30.10.2013
(73) Proprietor: Stora Enso Oyj, 00101 Helsinki (FI)
(72) Inventor: NÄSMAN, Mats, SE-652 30 Karlstad (SE); HARINEN, Marko, FI-01680 Vantaa (FI); TIMONEN, Olli, FI-554 00 Imatra (FI); RUOHONIEMI, Kimmo, FI-55100 Imatra (FI)
(74) Representative: Steinrud, Henrik
(86) International application number: PCT/SE2011/051534
(87) International publication number: WO 2012/087228

(56) References cited:
- WO-A1-94/20671
- WO-A1-2004/016850
- WO-A1-2006/072653
- CA-A1- 919 289
- US-A- 4 239 590
- US-A- 5 266 159
- US-A1- 2002 121 349
- US-A1- 2006 278 353
- PREIKSCHAT EKHARD: 'Measuring the Moisture and Bulk Density of Pulp Wood Chips for Digester Control - With a Correction Algorithm for Frozen Conditions' INSTRUMENTATION IN THE PULP AND PAPER INDUSTRY, PROCEEDINGS vol. 18, 13 May 1980 - 15 May 1980, ALBANY, NY, USA, pages 33 - 38, XP008170961

## Description

### Technical field

The invention refers to a method of controlling a pulping process wherein wood chips are conveyed to an impregnation vessel or to a digester where said wood chips are treated with a liquor comprising chemicals.

### Background

In a chemical pulping process, wood chips are treated with chemicals in a digester at enhanced pressure and temperature to dissolve the lignin that binds fibres together. The predominating pulping process today is the Kraft process, wherein wood chips are treated with a mixture of sodium hydroxide and sodium sulphide, known as white liquor.

The pulp quality and the consumption of the chemicals used in the pulping process are highly dependent on the raw material, i.e. the wood chips. The moisture content and other properties of the chips may vary due to, e.g., seasonal variations, different chip pile arrangements and the wood species used. The variation of the properties of the raw material makes it difficult to set an accurate dosing of chemicals to the digester. Oftentimes more chemicals than required are used, which is detrimental from both an economical and an environmental perspective.

A system for controlling a continuous digester is further disclosed in CA919289.

WO9420671 discloses a method to control a manufacturing process for pulp by measuring the bulk density of the chips supplied to the process.

US2006278353 discloses a method to monitor the variation in wood species composition by using light-reflection-related and density-related properties as input in a model characterizing a relation between such wood chip properties and species information.

In conventional chemical pulping processes, the process is controlled on the basis of information obtained from measurements of the properties of the pulp or of the residual alkali content in spent cooking liquor, i.e. the process is controlled in a feed-back manner. Such an approach fails to comply with short-term or sudden variations of the properties of the chips. In the art, there are commercial measurement systems available for measuring raw material properties. However, these prior art methods usually involve high investment costs, requires long time for analysis and/or are not accurate enough and are thus not typically used to control the process.

Thus, there remains a need for a simple, on-line feed forward control of the pulping process.

### Summary of the invention

It is an object of the invention to provide a simple, on-line method for controlling a pulping process. This, and other advantages, is achieved with the method according to the invention.

The invention discloses a method of controlling a pulping process wherein wood chips are conveyed to an impregnation vessel and/or to a digester where said wood chips are treated with a liquor comprising chemicals. The method of the invention comprises the steps of;
**a.** estimating a mass flow of dry wood chips to the impregnation vessel or the digester needed to achieve a desired pulp production, which estimated mass flow is achieved by dividing the desired pulp production with an estimated cooking yield,
**b.** measuring the actual mass flow of moisture wood chips conveyed to the impregnation vessel or the digester, by use of a chip conveyor scale, a mass flow scanner or a radiating wood flow meter,
**c.** calculating a ratio between the measured actual mass flow of moisture wood chips and the estimated mass flow of dry wood chips,
**d.** controlling the pulping process based on said calculated ratio.

The method according to the invention makes it, e.g. possible to control the supply of chemicals, such as sodium hydroxide and sodium sulphide, to the impregnation vessel or to the digester, the liquor to wood ratio and/or the pulping temperature on-line, in a feed-forward manner. It has been shown, that by controlling the pulping process in accordance with the invention, the stability of the process is improved and a reduction in the variation of the kappa number and the quality of the pulp is achieved. The method is simple and does not require huge investment costs. Further we are using the estimation in a) to calculate the pre-set process parameters. The ratio is then used for fine tuning the process parameters. Thus you create first a set-point which later is used in the regulation of the process.

### Detailed description of the invention

The invention relates to a method of controlling a pulping process wherein wood chips are treated with chemicals in an impregnation vessel and/or in a digester. The term "impregnation vessel" as used herein may be any kind of a vessel, pipe or the like suitable for processing of the wood chips. The pulping process may, e.g., be a kraft pulping process, a sulphite pulping process or a chemi-thermo mechanical pulping process. The pulping process may be a batch or a continuous pulping process. The process may, e.g., be a continuous Kraft pulping process, wherein the wood chips are treated with a mixture of sodium hydroxide and sodium sulphide at elevated temperature and pressure.

In accordance with the method of the invention, a ratio between the actual mass flow of fresh, moisture wood chips conveyed to the impregnation vessel or to the digester and an estimated mass flow of dry wood chips to the impregnation vessel or the digester needed to achieve a desired, pre-set, pulp production, is calculated. Said ratio, below referred to as Wood Material Indicator (WMI), may, e.g., be used to control the amount of chemicals, such as sodium hydroxide and sodium sulphide, supplied to the impregnation vessel or the digester and/or to control the liquor to wood ratio in the digester and/or to control the pulping temperature. The WMI may be calculated in accordance with eq. 1. $WMI = \frac{Actual mass flow of moisture chips \left[kg/s\right]}{Estimated mass flow of dry chips \left[kg/s\right]}$

Alternatively, the WMI may be calculated by dividing the estimated mass flow of dry wood chips with the actual mass flow of moisture wood chips.

An estimated mass flow of dry wood chips may be calculated by dividing the desired pulp production with the cooking yield in accordance with equation 2. $Estimated dry mass flow \left[kg/s\right] = \frac{pulp production}{Cooking Yield} \times 100$

The Pulp Production is a targeted, pre-set, value. The Pulp Production in the equation above is expressed in bone dry weight [kg/s], i.e. the weight of 100 % dry pulp. The cooking yield is an estimated value of the cooking yield for the wood species that are being pulped. The estimated cooking yield for kraft pulping of soft wood is, e.g., 46%.

The mass flow of moisture wood chips conveyed to the impregnation vessel or the digester is measured by use of a chip conveyor scale (preferred), a mass flow scanner (by using X-ray) or a radiating wood flow meter. The measured mass flow of moisture wood varies depending on the moisture content of the raw material and on other properties, such as the density, of the raw material.

The Wood Material Indicator (WMI) may be used to continuously control the pulping process. This may, e.g., be achieved by regulating the chemical charge to the impregnation vessel or the digester and/or the Liquor to wood ratio and/or the pulping temperature. The cooking alkali dose may be continuously regulated based on the WMI value. The Liquor to wood ratio may be regulated based on WMI by adjusting the internal circulation of spent cooking liquor or washing liquor in the digester.

When the variation in raw material density is higher the wood material indicator can be used in combination with frequent analysis of the dry content of the chips conveyed to the digester as reflected by the third aspect of the present invention.

In such a way the possible variation from humidity and raw material density is separated from each other and this will further improve the precision of the process control if the variation in mass flow is dominated by raw material density variation. This is decided case by case on the conditions in the mill and used raw material.

The estimated dry mass flow is calculated by eq.2. The production in a continuous digester system is normally controlled by a volumetric measurement such as a chip feeding screw or a chip meter. Based on the known feeding volume per revolution, filling degree and estimated chip density the chip feeding device will rotate with a certain speed in order to maintain the target production (estimated dry mass flow). By utilising the measured wet chip flow measured on the chip conveyor to the digester system in combination with an analysed chip dry content and the known volume (given by the rotation speed of the chip metering device) of chips fed to the digester system it is possible to calculate the measured wet chip density: $Wet chip density = WCF / \left(V\times FD\times rpm\right)$

Where
WCF = wet chip mass flow (kg/min)
V = fed volume per revolution (m³)
FD = filling degree
rpm = rotation speed of the chip metering devise (rpm)

The measured dry density is then calculated from: $Measured dry density = wet chip density \times dry content .$

In this case the WMI is defined as $WMI = Measured dry density / estimated dry density$

WMI as described by the ratio above may then be used in the process control. The estimated dry density is dependent on which raw material is used.

Further the method according to the invention is used in a feed forward loop (manner) taking into account what is fed into the system (variation in both dry matter and moisture is combined; in the Nordic conditions where variation in chip bulk density is very low this has worked well). The response to changes is further relatively fast.

In the following the invention will be described in more details by way of an example with reference to the drawings.

### Description of the drawings

Fig. 1 shows a schematic view of the flow of wood raw material from a chip pile to an impregnation vessel or to a digester. Total mass flow is measured preferably by using a chip conveyor scale. The raw material of fresh, moisture wood chips is conveyed on a chip conveyor (1) to a chip silo (2). The material is further conveyed from the chip silo (2) to an impregnation vessel or a digester by use of a chip feed screw (3). The screw rotation of the chip feed screw (3) is controlled based on the calculated estimated dry mass flow, i.e. it depends on the set value of the pulp production. According to one example of the invention, a chip conveyor scale (4), arranged under the chip conveyor (1), measures the actual flow of fresh, moisture chips continuously. Since the mass of chips in the silo is held substantially constant, measuring of the flow on the chip conveyor gives an accurate value of the actual flow of fresh, moisture chips to the impregnation vessel or the digester. The measured fresh flow value is transmitted to a control unit (5) of a control system, (5) shown schematically in fig. 3. The estimated dry wood flow is also entered into the control unit (5). In the control system, a ratio between said flows is calculated (WMI) and used to regulate e.g. the set value for the alkali charge to the impregnation vessel or the digester and the liquid to wood ratio. Preferably, the process is further controlled on the basis of a theoretically calculated flow of wood chips to the impregnation vessel or the digester, i.e. in accordance with the traditional way of controlling a pulping process. Thus, WMI is preferably used to regulate a certain percentage on top of the traditional control of the process. A theoretically calculated set value (set-point) is thus also entered into the system.
Figure 2 shows an example how the WMI as set out above may be determined.
Figure 3 shows a control system in accordance with the invention. The control system may comprise one or several sub control systems for regulating the alkali charge, cooking temperature and/or Liquor to wood ratio for long term, e.g. 24 hours, and/or short term, e.g. 2 hours, variations of the WMI. In the control system (5) shown in fig. 3, the regulation is separated into two circuits; one for long term and one for short term variation of WMI. The system (5) may comprise further control units (6, 7) where further variables (v1, v2, ... Vn) or preset values may be entered for controlling the process, such as the upper and lower limits of alkali charge, the current values of the liquor to wood ratio, cooking temperature (H-factor) and alkali charge etc.
Figure 4 shows more schematic how WMI according to the present invention may be used to control alkali dosage, which is only an example of a parameter which may be controlled by using the WMI according to the present invention.
Figure 5 shows the WMI control in action (c.f. the example below).

### Example

A trial run was performed at the Oulu mill during 4 days where it was shown that WMI control reduces kappa variation. WMI as a soft sensor appears to be usable and accurate enough to reduce the effects of raw material variations. The results are given below in Table 1.

**Table 1. Results from the 4-day Oulu trial. Each case is a period of 4d running. The raw material was softwood of Scandinavian origin (t/d=tonnes/day). See also figure 5 which reflects the example. C.f. also figure 2.**

| | | No WMI control | | | | With WMI control | | | |
|---|---|---|---|---|---|---|---|---|---|
| Measurement | Unit | Average | Deviati on | Maxim um | Minim um | Average | Deviati on | Maxim um | Minim um |
| Alkali to wood ratio | % | 19.1 | 0.10 | 19.2 | 19.0 | 19.0 | 0.05 | 19.2 | 18.8 |
| Residual alkali extraction [g/l] (average 2h) | g/l | 6.1 | 0.27 | 6.8 | 5.4 | 5.8 | 0.21 | 6.6 | 5.2 |
| WMI value as % of DC in wood (average 2h) | % | 47.7 | 0.47 | 48.7 | 46.9 | 48.0 | 0.41 | 49.0 | 47.3 |
| On-line blow kappa value from analyzer | | 27.1 | 1.27 | 31.5 | 24.4 | 26.7 | 0.74 | 28.8 | 25.0 |
| Cooking temperature | °C | 167.6 | 0.53 | 168.6 | 166.0 | 169.0 | 0.72 | 171.0 | 167.0 |
| Cookinq production | t/d | 1123 | 6.98 | 1127 | 1099 | 1150 | 0.16 | 1150 | 1149 |

The benefits are given below in Table 2.

**Table 2. The benefits from the 4-day Oulu trial.**

| **Benefits of using wood material indicator (WMI) control** | |
|---|---|
| Change in residual alkali variation (black liquor extraction) | -22.1 % |
| Change in kappa variation (after digester blow) | - 41.7 % |

Various embodiments of the present invention have been described above but a person skilled in the art realizes further minor alterations, which would fall into the scope of the present invention. The breadth and scope of the present invention should not be limited by any of the above-described exemplary embodiments, but should be defined only in accordance with the following claims and their equivalents. Other aspects, advantages and modifications within the scope of the invention will be apparent to those skilled in the art to which the invention pertains. Thus the invention is therefore intended to cover various modifications and equivalent methods included within the spirit and scope of the appended claims.

Any illustration and description in the drawings and in the foregoing description are to be considered exemplary and not restrictive.

Use of the word "comprising" in the claims does not exclude other elements or steps, and use of the article "a" or "an" does not exclude a plurality. Occurrence of features in different dependent claims does not per se exclude a combination of these features. Any reference signs in the claims are for increasing intelligibility and shall not be construed as limiting the scope of the claims.

## Claims

1. A method of controlling a pulping process wherein wood chips are conveyed to an impregnation vessel and/or to a digester where said wood chips are treated with a liquor comprising chemicals, which method comprises the steps of;
**a.** estimating a mass flow of dry wood chips to the impregnation vessel or to the digester needed to achieve a desired pulp production, which estimated mass flow is achieved by dividing the desired pulp production with an estimated cooking yield,
**b.** measuring the actual mass flow of moisture wood chips conveyed to the impregnation vessel or to the digester by use of a chip conveyor scale, a mass flow scanner or a radiating wood flow meter,
**c.** calculating a ratio between the actual mass flow of moisture wood chips and the estimated mass flow of dry wood chips,
**d.** controlling the pulping process based on said calculated ratio.

2. A method according to claim 1, wherein the step (d) of controlling the pulping process comprises controlling the chemicals supplied to the impregnation vessel and/or to the digester based on said calculated ratio.

3. A method according to any one of claims 1 - 2, wherein the step (d) of controlling the pulping process comprises controlling the liquor to wood ratio in the digester based on said calculated ratio.

4. A method according to anyone of claims 1 - 3, wherein the step (d) of controlling the pulping process comprises controlling the pulping temperature based on said calculated ratio.

## Patentansprüche

1. Verfahren zum Steuern eines Aufschlussprozesses, bei dem Holzspäne zu einem Imprägniergefäß und/oder einem Kocher gefördert werden, wo die Holzspäne mit laugenenthaltenden Chemikalien behandelt werden, wobei das Verfahren folgende Schritte umfasst:
**a.** Abschätzen des Massenflusses der trockenen Holzspäne zum Imprägniergefäß oder Kocher, der nötig ist, um eine gewünschte Zellstoffproduktion zu erreichen, wobei der geschätzte Massenfluss durch Aufteilen der gewünschten Zellstoffproduktion mit einer geschätzten Kochausbeute erreicht wird,
**b.** Messen des tatsächlichen Massenflusses der feuchten Holzspäne, die zum Imprägniergefäß oder Kocher gefördert werden, durch Verwendung einer Spanförderwaage, eines Massenflussscanners oder eines strahlende Holzsflussmessgeräts,
**c.** Berechnen eines Verhältnisses zwischen dem tatsächlichen Massenfluss der feuchten Holzspäne und dem geschätzten Massenfluss der trockenen Holzspäne,
**d.** Steuern des Aufschlussprozesses auf Basis des berechneten Verhältnisses.

2. Verfahren nach Anspruch 1, wobei der Schritt (d) des Steuerns des Aufschlussprozesses das Steuern der Chemikalien umfasst, die dem Imprägniergefäß und/oder dem Kocher auf Basis des berechneten Verhältnisses zugeführt werden.

3. Verfahren nach einem der Ansprüche 1 - 2, wobei der Schritt (d) des Steuerns des Aufschlussprozesses das Steuern des Verhältnisses zwischen Lauge und Holz im Kocher auf Basis des berechneten Verhältnisses umfasst.

4. Verfahren nach einem der Ansprüche 1 - 3, wobei der Schritt (d) des Steuerns des Aufschlussprozesses das Steuern der Aufschlusstemperatur auf Basis des berechneten Verhältnisses umfasst.

## Revendications

1. Procédé de contrôle d'un processus de trituration dans lequel les copeaux de bois sont transmis dans un récipient d'imprégnation et/ou dans un digesteur où lesdits copeaux de bois sont traités à l'aide d'une liqueur constituée de produits chimiques, ledit procédé comprenant les étapes consistant à ;
**a.** l'estimation d'un flux de masse de copeaux de bois secs dans le récipient d'imprégnation ou le digesteur nécessaire à la production d'une quantité souhaitée de pâte, ce qui est obtenu en divisant la production de pâte désirée par un rendement de cuisson estimé,
**b.** la mesure du flux de masse réel des copeaux de bois humides acheminés dans le récipient d'imprégnation ou dans le digesteur à l'aide d'une échelle de convoyeur à copeaux, d'un analyseur de flux de masse ou d'un détecteur de débit de bois rayonnant,
**c.** le calcul d'un rapport entre le flux de masse réel des copeaux de bois humides et le flux de masse estimé des copeaux de bois secs,
**d.** le contrôle du processus de mise en pâte en fonction du rapport calculé.

2. Procédé selon la revendication 1, dans lequel l'étape (d) de contrôle du processus de mise en pâte consiste à contrôler les produits chimiques fournis au récipient d'imprégnation et/ou au digesteur en fonction dudit rapport calculé.

3. Procédé selon l'une quelconque des revendications 1 - 2, dans lequel l'étape (d) de contrôle du processus de mise en pâte consiste à contrôler le rapport de la liqueur au bois dans le digesteur en fonction du rapport calculé.

4. Procédé selon l'une quelconque des revendications 1 - 3, dans lequel l'étape (d) de contrôle du processus de mise en pâte consiste à contrôler la température de la pâte en fonction du rapport calculé.
